

## UNITED STATES PATENT OFFICE

2,164,393

## LUBRICATING OIL

Elliott Alfred Evans, London, England, assignor  
to C. C. Wakefield & Company Limited, Lon-  
don, England, a British company

No Drawing. Application April 14, 1936, Serial  
No. 74,388. In Great Britain April 15, 1935

12 Claims. (Cl. 87—9)

This invention is for improvements in or relating to lubricants which are to be used under conditions which tend to disrupt the lubricant film, which disruption more particularly takes place when the pressure between the bearing surfaces is very great.

Where the lubricant is required to lubricate surfaces under the above conditions, the film-rupture strength becomes more important than the coefficient of friction. For example, under the extreme pressures obtaining in hypoid gears, if the oil film is ruptured, the metal surfaces will contact one with the other, thereby leading to loss of efficiency, excessive wear and failure of the mechanism.

There have already been provided lubricants which have a high film-rupture strength, for example, of the order of 10,000 pounds per square inch and such lubricants are generally known in the trade as "extreme-pressure" lubricants. On the other hand, an ordinary lubricating oil has a film-rupture of about 3,000 to 4,000 pounds per square inch.

These extreme-pressure lubricants originally consisted of lubricating oil which contained sulphur, either in the form of flowers of sulphur or as a colloidal dispersion. The sulphur, however, was liable to precipitation and it was later proposed to prepare these extreme-pressure lubricants by treating a fatty oil, for example an animal oil, with thionylchloride or with similar reagents, such as sulphur monochloride, sulphur dichloride etc., and then adding the product of this reaction to a mineral oil.

The theory as to the action of extreme-pressure lubricants has been that the sulphur reacts with metallic surfaces and forms a very thin coating of iron sulphide and that this sulphide film is sufficient to prevent the metallic surfaces coming into contact with one another should the lubricant film be ruptured. If this theory is, in fact, correct, then it is obvious that the sulphur contained in the oil must be in such form as to be capable of reacting with the metallic surfaces which it is desired to lubricate. On the other hand, the sulphur compound must not be so reactive as to induce corrosion of the surfaces.

It was found, however, that with these prior processes no set conditions could be determined which would ensure a uniform product always being obtained and it was therefore always necessary when preparing an extreme-pressure lubricant to apply the method of trial and error in arriving at a satisfactory composition.

It will be appreciated, therefore, that in order

to overcome these difficulties it is desirable to utilise as far as possible definite compounds, of high purity, in order that reproducible results may be obtained without resorting to the laborious and probably inaccurate method of trial and error.

According to this invention an extreme-pressure lubricant comprises a lubricating oil or grease having dispersed therein a small quantity of a thio-ether. It has been found that the desired effects may be obtained by employing the thio-ether in quantities up to about 2% by weight of the oil.

A feature of the invention consists in that the thio-ether comprises two aromatic radicals. Preferably, at least one of said aromatic radicals contains either a hydroxyl substituent or a carboxyl (or ester) substituent.

A further feature of the invention consists in that each of said aromatic radicals contains both a hydroxyl substituent and a carboxyl (or ester) substituent. Preferably, the hydroxyl substituents are located in the para-position in the aromatic radical.

A still further feature of the invention consists in that said thio-ether contains two aliphatic radicals. Either one or both of said aliphatic radicals contains either an hydroxyl substituent or a carboxyl (or ester) substituent or both.

In one preparation which is given by way of example, a mixture of 50 grams of thionylchloride and 30 grams of methyl-salicylate was placed in a 300 cc. flat-bottomed flask and 20 grams of copper dust were then slowly added. The reaction which then takes place is accompanied by the generation of heat and the evolution of fumes of sulphur dioxide and hydrogen chloride; the reaction mixture is allowed to stand over-night and is then heated in a water bath for from one to two hours. The mixture is extracted with hot chloroform and the chloroform extract is filtered to remove sulphur, precipitated copper and other impurities; the product is finally obtained by concentration of the chloroform extract followed by recrystallisation. The material thus obtained is bis-(3-carbomethoxy 4-hydroxyphenyl) thio-ether.



5

10

15

20

25

30

35

40

45

When 0.5% of this pure compound was added to a pure mineral oil, the film-rupture strength was found to be raised to the extremely high

55

value of 15,000 pounds per square inch, a remarkable increase over the value obtained with the pure mineral oil which, in the Almen tester, gave a film-rupture strength of between 3,000 to 4,000 5 pounds per square inch. The extreme-pressure lubricants hitherto prepared have in general required at least 5% of a sulphur base (prepared by reacting sulphur chloride with the fatty oil) in order to produce a comparable increase in the 10 film rupture strength of the oil.

Other compounds which may be employed are those obtained, in an analogous manner to that described above, from ethyl benzoate and ethyl phthalate which when used in a mineral oil in 15 quantities of 1% have yielded lubricants having a film-rupture strength of 14,000 and 12,000 pounds per square inch respectively. The thio-ether prepared, in a similar manner to that described above, from ethyl crotonate when added 20 to a mineral oil in the proportion of 1% by weight yielded a lubricant having a film-rupture strength of 11,000 pounds per square inch. It will be understood that the thio-ethers may be prepared by any suitable method, for example, 25 they may be prepared by reacting sulphur monochloride or sulphur dichloride with the aliphatic or aromatic compounds instead of thionyl chloride.

The invention also includes within its scope, 30 the method of preparing extreme-pressure lubricants which comprises dispersing thio-ethers of the above-mentioned class in a lubricating oil or grease in quantities, which are accurately controllable.

35 It will also be appreciated that the invention is not restricted to the employment of particular proportions of the thio-ethers since within certain limits the film-rupture strength of the lubricant may be adjusted to a desired value in 40 accordance with the quantity of thio-ether added in order to render the lubricant suitable for any special use or mechanism.

I claim:

1. An extreme-pressure lubricant comprising a 45 lubricant having dispersed therein between 0.1% and 2% of a thio-ether comprising two aromatic radicals at least one of which aromatic radicals contain an ester substituent.

2. An extreme-pressure lubricant comprising a 50 lubricant having dispersed therein between 0.1% and 2% of a thio-ether comprising two aromatic radicals at least one of which aromatic radicals contains an hydroxyl substituent and an ester substituent.

3. An extreme-pressure lubricant comprising a lubricant having dispersed therein between 0.1% and 2% of a thio-ether comprising two aromatic radicals at least one of which aromatic radicals contains an hydroxyl substituent in the para- 5 position and an ester substituent.

4. An extreme-pressure lubricant comprising a lubricant having dispersed therein between 0.1% and 2% of a thio-ether comprising two aromatic radicals both of which aromatic radicals contain 10 an hydroxyl substituent in the para-position and an ester substituent.

5. An extreme-pressure lubricant comprising a lubricating oil having dispersed therein between 0.1% and 2% of a thio-ether having an 15 ester-substituent.

6. An extreme-pressure lubricant comprising a mineral lubricating oil having dispersed therein up to 2% of bis (3-carbomethoxy 4-hydroxy- 20 phenyl) thio-ether.

7. An extreme-pressure lubricant comprising a mineral lubricating oil having dispersed therein about 1% of the thio-ether formed by the condensation of ethyl benzoate in the presence of thionyl chloride and copper dust. 25

8. An extreme-pressure lubricant comprising a mineral lubricating oil having dispersed therein about 1% of the thio-ether formed by the condensation of ethyl phthalate in the presence of thionyl chloride and copper dust. 30

9. An extreme-pressure lubricant comprising a lubricant having dispersed therein between 0.1% and 2% of a thioether having a substituent-group—COOX wherein X is a radical of the group consisting of aliphatic radicals. 35

10. An extreme-pressure lubricant comprising a lubricant having dispersed therein between 0.1% and 2% of a thioether each radical of which contains a substituent-group—COOX in which X is of the group consisting of aliphatic 40 radicals. 40

11. A lubricant comprising a lubricating oil having dispersed therein an extreme-pressure agent consisting of a thioether having a substituent-group—COOX in which X is of the group 45 consisting of aliphatic radicals.

12. A lubricant comprising a lubricating oil having dispersed therein between 0.1% and 2% of an extreme-pressure agent consisting of a thioether each radical of which contains a substituent-group—COOX in which X is of the group 50 consisting of aliphatic radicals.

ELLIOTT ALFRED EVANS.